

# UNITED STATES PATENT OFFICE.

BENJAMIN H. DOSENBACH, OF BUTTE, MONTANA; EDNA M. DOSENBACH EXECUTRIX  
OF SAID BENJAMIN H. DOSENBACH, DECEASED.

## ORE-CONCENTRATION PROCESS.

1,377,189.

Specification of Letters Patent.

Patented May 10, 1921.

No Drawing.

Application filed November 16, 1917. Serial No. 202,268.

*To all whom it may concern:*

Be it known that I, BENJAMIN H. DOSEN-  
BACH, a citizen of the United States, resid-  
ing at Butte, in the county of Silver Bow  
5 and State of Montana, have invented certain  
new and useful Improvements in an Ore-  
Concentration Process, of which the follow-  
ing is a specification.

My invention is an improvement in that  
10 form of the flotation process wherein the  
modifying agent is introduced into the ore  
pulp in the gaseous form and generally in  
admixture with some other gas such as air.  
By the term "modifying agent" I refer to  
15 the substance used for the purpose of pro-  
moting the preferential attraction of the  
gaseous bubbles for certain constituents of  
the ore as distinguished from other con-  
stituents. When the modifying agent is in-  
20 introduced into the ore pulp in the gaseous  
form by mechanical agitation or through a  
porous medium such as canvas, unglazed  
earthenware, concrete or other porous mate-  
rial, the gaseous modifying agent may either  
25 be the vapor of a substance that normally  
assumes the liquid or solid form, that is, that  
assumes the liquid or solid form at the ordi-  
narily prevailing temperatures and pres-  
sures or the gaseous modifying agent may  
30 be a permanent gas, that is, a substance  
which normally exists in the gaseous form  
at ordinary temperatures and pressures. A  
great variety of substances may be used as  
35 modifying agents in the gaseous form, such  
as the products formed by gasifying many  
ordinary oils, pine oil, oleic acid, etc., coal  
and wood tar and derivatives thereof and the  
gases formed by the distillation of a wide  
40 variety of organic substances such as wood,  
coal, asphaltic matter and gilsonite. My in-  
vention is not restricted to use in connec-  
tion with any particular gaseous modifying  
agent.

I have found that when an ore contains  
45 several metalliferous constituents such as the  
sulfids of iron, zinc and lead certain of the  
metalliferous constituents may be floated  
to the almost complete exclusion of the  
others by the use of certain reagents which  
50 have a deterrent effect upon the flotation of  
some of the sulfid constituents but not upon  
others. The agent used for preventing the  
flotation of some of the metalliferous con-  
stituents may be either some salt or other  
55 substance added to and mixed with the ore

pulp into which the gaseous modifying agent  
is introduced, or, in other instances may be  
some gas or vapor mixed with the modify-  
ing gas before it is introduced into the pulp.  
For instance, in the case of an ore contain-  
ing sulfids of iron together with galena and  
blende, the admixture of sulfur dioxid in  
proper amounts with the gaseous modifying  
agent has the effect of preventing the floata-  
tion of the blende while not interfering with  
the flotation of the galena. The amount of  
sulfur dioxid to be used in admixture with  
the gaseous modifying agent can only be de-  
termined by experimentation upon the par-  
ticular ore being treated. Even in the case  
60 of a particular ore a quantitative deter-  
mination by volume of the proportion of  
sulfur dioxid to modifying gas is difficult,  
but the regulation itself is comparatively  
simple if the sulfur dioxid be discharged  
65 into the current of modifying gas through  
a regulating valve or other controlling  
means. A satisfactorily sharp separation of  
blende from the sulfid of iron and galena  
70 can be effected by the means described and  
the residue containing the blende can subse-  
quently be concentrated by flotation treat-  
ment, the effect of the sulfur dioxid in pre-  
venting the flotation of the blende being only  
75 temporary.

Under certain conditions sulfuric acid in  
small amounts when added to the ore pulp  
likewise causes preferential flotation of one  
metalliferous constituent of a mixed ore as  
distinguished from other constituents. For  
80 instance, in treating an ore containing sul-  
fids of lead and zinc, a small amount of sul-  
furic acid almost completely prevents the  
flotation of the zinc sulfid, while not inter-  
fering with the flotation of the lead sulfid,  
85 and a subsequent treating of the residue un-  
der other conditions will bring about the  
flotation of the zinc sulfid.

Sodium hydrate or the hydrate of alkaline  
or alkaline earths when added to a pulp of  
zinc lead ore without acid has the effect,  
upon the introduction of the modifying gas,  
of preventing the flotation of the zinc while  
not interfering with the flotation of the lead  
and the zinc contained in the residue can be  
105 floated in the subsequent operation in which  
sulfuric acid is added to the pulp.

Sodium sulfhydrate ( $\text{NaSH}$ ) has an ac-  
tion similar to that of sodium hydrate as a  
deterrent upon flotation of zinc sulfid in the

60

65

70

75

80

85

90

95

100

105

110

presence of lead sulfid and gangue. Other soluble sulfur compounds and a variety of other substances have a similar deterrent effect upon the flotation of part of the metalliferous constituents of mixed ores and my invention includes the use of a gaseous modifying agent, either a permanent gas or the vapor of a normally liquid or soluble substance tending to bring about flotation 10 of all of the metalliferous constituents of an ore together with the use of some deterrent agency acting to more or less completely prevent the flotation of part of the metalliferous constituents, such deterrent agency 15 taking the form either of some gas mixed with the modifying gas or some substance added to and mixed with the ore pulp.

What I claim is:

1. In a process of flotation concentration 20 of ores containing a plurality of floatable metalliferous constituents the operations of introducing into the ore pulp a gaseous modifying agent tending to cause flotation of all of said constituents and simultaneously introducing a gaseous substance 25 which has a deterrent effect upon the flota-

tion of some of the metalliferous constituents of the ore but not upon others.

2. In a process of flotation concentration 30 of ores containing a plurality of floatable metalliferous constituents the operations of introducing into the ore pulp a gaseous modifying agent tending to cause flotation of all of said constituents mixed with a gaseous substance which has a deterrent effect 35 upon the flotation of some of the metalliferous constituents of the ore but not upon others.

3. In a process of flotation concentration 40 of ores containing a plurality of floatable metalliferous constituents the operations of introducing into the ore pulp fine streams of a gaseous modifying agent tending to cause flotation of all of said constituents mixed with a gaseous substance which has a 45 deterrent effect upon the flotation of some of the metalliferous constituents of the ore but not upon others.

In testimony whereof, I have subscribed my name.

BENJAMIN H. DOSENBACH.